

1

3,293,896

**COATED METAL ARTICLE AND METHOD  
OF MAKING SAME**

Andrew J. Kompanek, Jr., Lansdale, Pa., assignor to  
Teleflex Incorporated, North Wales, Pa., a corporation  
of Delaware  
No Drawing. Filed June 28, 1963, Ser. No. 291,267  
5 Claims. (Cl. 72—47)

The subject matter of the present invention is an improved corrosion resistant shaped metal article, and method for making same.

It is presently conventional practice to form many types of metal articles to substantially final shape by cold forming operations such as cold extrusion. Typical of articles so manufactured are valves and valve stems, ball studs, switch housings, spark plug shells and the like. The billet used for the extrusion or other cold forming operation can be either cut from ball stock or, as is becoming more the practice, it can be formed of compacted sintered metal powder.

Many of the steel or other ferrous base articles manufactured by such techniques are required to have oxidation and other corrosion resistance in their final form. For example, valves must be highly resistant to erosion or corrosion by combustion gases and switch casings and spark plug shells must often have at least a certain amount of resistance to rusting. The conventional practice is to surface treat the formed metal articles in order to provide such corrosion resistance. Frequently, the nature of the finished article is such that really good corrosion coating is not economically feasible and hence bluing, phosphating or other inexpensive treatments are used merely to provide a pleasing initial appearance and corrosion resistance, which is effective only during the initial period of use. In the case of spark plug shells, for example, a relatively inexpensive surface treatment is used where the plugs are for automotive use with the result that rusting generally occurs after only a few weeks. For marine spark plugs where more durable resistance to salt corrosion and the like is essential, cadmium plating treatments or the like must be used but at considerable additional expense.

It is a principal object of the present invention to provide a method for cold forming metal articles wherein during such forming method the article is provided with a highly corrosion resistant surface finish which can be of pleasing lustrous metallic appearance, if desired. Another and attendant object of the invention is the provision of an improved low cost formed metal article having a corrosion resistant surface finish.

Briefly, the aforesaid objects are accomplished in accordance with the invention, by extruding or otherwise cold forming a metal billet having a surface layer which is provided by coating the billet with a uniform slurry of a finely divided solid particulate material in an aqueous solution containing major or substantial amounts of phosphate ion, metal ion, and ion selected from the group consisting of chromate, molybdate and mixtures thereof. The solid particulate material can, for example, be a metal powder such as powdered aluminum, nickel and silver, aluminum being much preferred, or it can be a finely divided dry lubricant such as molybdenum disulfide, tungsten disulfide, graphite or lead oxide. Frequently it will be desirable to use combinations of different solid particulate materials, for example, aluminum powder in combination with a powdered dry lubricant.

No claim is herein made to the coating composition per se, such being covered by United States patent applications S.N. 291,269, S.N. 291,271, S.N. 291,289 and S.N.

2

291,248, all of said applications being assigned to the assignee of the present invention.

The phosphate anion concentration should preferably be from 1 to 4 mols per liter though as little as .5 per liter is satisfactory for some applications of the coatings. The phosphate can be introduced into the solution in the form of phosphoric acid, in the form of phosphates of the metal or metals to be included as the metal cation or, as is preferred, it can be added in both forms. It will be understood that the term "phosphate" is intended to comprehend not only the  $\text{PO}_4$  ion but also the  $\text{HPO}_4$  and  $\text{H}_2\text{PO}_4$  ions. All three, for example, result from the ionization of  $\text{H}_3\text{PO}_4$  and the hydrogen phosphate ions generally will, at least to some extent, be present in the compositions of this invention. Where phosphoric acid is used as additive in making the compositions, it is much desired to use the ortho acid  $\text{H}_3\text{PO}_4$  though the invention also comprehends the use of the other forms such as the metal or pyro acids all ionizing in water to provide phosphate anion. Examples of metal phosphates which can be used to add phosphate ion are the mono, di and tribasic phosphates of magnesium, zinc, aluminum, iron and lithium. The phosphate used should, of course, be soluble in the solution though this does not mean it must be highly water soluble since many of the phosphates not soluble in water are nevertheless soluble in an acid solution, for example, one containing phosphoric acid or chromic acid. In general, however, the mono and dibasic phosphates, which are more soluble than the tribasic salts, are preferred. The chromate ion concentration should be from about .3 to 3 mols per liter, at least .5 mol per liter being preferred. The chromate can be added as chromic acid, or as a metal chromate or dichromate, for example, the chromate or dichromate of magnesium, zinc, aluminum, calcium, barium, lithium, sodium or silver. If it is desired, to replace the chromate ion in whole or in part with molybdate ion, molybdic acid or the metal molybdates, for example, zinc molybdate can be used. Chromate ion is, however, preferred.

The metal ion concentration should be from about .2 to 4 mols per liter and preferably at least about 1 mol per liter. Where the phosphate and/or chromate or molybdate ion is furnished to the solution by addition of a metal salt, in accordance with the above, this inherently also supplies metal ion to the solution, hence, any of the aforementioned phosphates, chromates, dichromates or molybdates can be used as the source of metal ion. Additionally, metal ion can be supplied in the form such as metal oxide, hydroxide, carbonate, etc. which will dissolve in acid to produce the metal phosphate, chromate, or molybdate and therefore the metal ion, plus water and/or gas which is evolved. Of course, if the metal ion is added in this form the other solution additions must supply the acidity required to accomplish the acid-base reaction. For example, some of the phosphate ion should be added as phosphoric acid, as is preferred, or some of the chromate as chromic acid. The following metal compounds will illustrate those which can be added to generate the metal ion within the solution in accordance with the above: Magnesium oxide, magnesium hydroxide, zinc hydroxide, aluminum hydroxide, lithium oxide, lithium carbonate, calcium hydroxide, calcium carbonate. Of course, it will be understood that the insoluble refractory metal oxides, for example alumina, which can be used as the solid particulate material in the practice of this invention as hereinafter described, cannot be employed as the metal ion additive since they are difficult if not impossible to dissolve even in the strong acid.

In general, the valence +2 and +3 metals are preferred. Magnesium is outstanding though for some specific uses of the compositions, the ferric and aluminum

ions which are +3 valence, will serve to advantage. While not as good as magnesium, zinc is also desirable. The valence +1 metals are satisfactory though for most applications of the coatings it is generally preferable to use them only in combination with valence +2 and/or valence +3 metals.

The solid particulate material should preferably have a grain size of less than 325 mesh and should, of course, be insoluble in the solution and hence form a slurry therewith. It can be included in an amount of from 10 to 2000 grams per liter though for most uses from about 200 to 800 grams per liter will be preferred. Examples of solid particulate materials are the metal powders, such as powdered aluminum, nickel and silver, aluminum being outstandingly advantageous, and the dry lubricants such as molybdenum disulfide, tungsten disulfide, graphite and lead oxide.

To attain a coating with exceptionally good lubricity and flexibility, the organic polymers of high inherent lubricity, ideally polytetrafluoroethylene, can be included in place of or in addition to the solid particulate material as described and covered by U.S. applications S.N. 291,248 and S.N. 291,358 filed concurrently herewith and assigned to the assignee of the present invention.

In practice, the metal billet is first coated with the slurry of the particulate material in the phosphate-metachromate and/or molybdate ion solution and then dried and preferably cured by heating to a temperature and for a time sufficient to cause the coating to become water insoluble. Then the coated billet is cold formed to desired shape as by extrusion. The coating flows and stretches with the metal without cracking or otherwise disintegrating with the result that the shaped article has a thin surface film of the cured mixture. Due to the working of the metal and the coating material during such forming operation, the coating is somewhat diffused into the metal and takes on properties even superior to those prior to such working. The thickness of the coating applied to the billet can be from .0005 to .02 inch, the precise optimum thickness depending upon the amount of metal flow in the forming operation. That is, the initial coating should be thick enough to assure a continuous coating on the finished article. If desired, two or more coats may be applied. If metal powder, ideally aluminum, is used as the solid particulate material, the shaped article can be buffed to provide a lustrous pleasing metallic appearance. The coating is highly corrosion resistant and by the choice of particulate material, other desirable properties such as abrasion resistance or lubricity can additionally be imparted. Where the coating includes a dry lubricant, the method has the additional advantage of increasing tool life. Because of the excellent flexibility of the coating, finishing operations such as thread rolling or the like can be used without disrupting the coating.

If desired the curing operation can be accomplished after rather than prior to the cold forming operation. This has a disadvantage, however, in that more careful handling of the coated billet is required since the uncured coating has incomparably less strength than the cured coating and hence can be scratched off in the course of rough conveying operations prior to forming and curing.

The following specific examples of the coatings will serve to further illustrate.

#### Example 1

|                                          |        |      |
|------------------------------------------|--------|------|
| $H_3PO_4$ (85% aqueous solution) -----   | cc.    | 200  |
| $MgO$ -----                              | grams. | 50   |
| $Mg(H_2PO_4)_2 \cdot 3H_2O$ -----        | do     | 50   |
| $MgCr_2O_7 \cdot 6H_2O$ -----            | do     | 160  |
| Aluminum powder (spherical, 5-10 micron) |        |      |
| do                                       | 800    |      |
| Water, to -----                          | cc.    | 1000 |

75

#### Example 2

|                                            |       |      |
|--------------------------------------------|-------|------|
| $CrO_3$ -----                              | grams | 100  |
| $AlPO_4$ -----                             | do    | 122  |
| $H_3PO_4$ -----                            | do    | 98   |
| 5 Aluminum powder (spherical, 5-10 micron) |       |      |
| do                                         | 600   |      |
| Molybdenum disulfide (5-10 micron) -----   | do    | 100  |
| Water, to -----                            | cc    | 1000 |

10

#### Example 3

|                                              |       |      |
|----------------------------------------------|-------|------|
| $H_3PO_4$ (85% aqueous solution) -----       | cc    | 150  |
| $ZnCrO_4$ -----                              | grams | 40   |
| $MgCr_2O_7 \cdot 6H_2O$ -----                | do    | 60   |
| 15 $Mg(H_2PO_4)_2 \cdot 3H_2O$ -----         | do    | 60   |
| Teflon dispersion, aqueous (60% solid) ----- | cc    | 400  |
| Aluminum powder (spherical, 5-10 micron)     |       |      |
| grams                                        | 600   |      |
| Water, to -----                              | cc    | 1000 |

20

The steel or other metal billet is first thoroughly cleaned and is then coated as by spraying or dipping with a composition such as one of the above. Then the coated billet is dried and cured to complete water insolubility, the precise curing temperature and time depending upon the composition being used. In general, the curing temperature will be from 500 to 800° F. and the time of cure from 3 to 60 minutes. The lower the temperature, the more time required to accomplish a full cure. If a lower curing temperature is necessary or desirable, coating compositions as covered by United States patent applications S.N. 291,268 and S.N. 291,270, now Pat. Nos. 3,248,249 and 3,248,250, respectively, assigned to the assignee of the present invention, can be used. Briefly, such coatings are the same as those described above except that they additionally include from about 1 to 100 grams per liter of a soluble metal silicate preferably sodium silicate or a colloidal grain size inorganic gel former such as silica gel or alumina gel, or a combination thereof. With such additives, temperatures of from 250 to 500° F. can be used to accomplish a full cure.

The coated and cured billet can then be formed to desired final shape by any of the conventional cold forming techniques such as extrusion. By "cold forming" is meant forming at room temperature or at least at temperatures, i.e. with a billet temperature, not exceeding about 1000° F. though higher temperature may, of course, occur for a very short period during actual metal movement.

50 While the invention has been described specifically with reference to certain embodiments thereof, various changes and modifications may be made all within the full and intended scope of the claims which follow.

I claim:

1. A method for forming a metal article of predetermined shape with a corrosion resistant coating thereon including the steps of coating a metal billet with a mixture of a solid particulate material and an aqueous solution, the solute of said aqueous solution consisting essentially of a combination of inorganic compounds selected from the group consisting of phosphoric acid, chromic acid, molybdic acid, and the metal salts of said acids, the combination of compounds in said aqueous solution being such as will provide at least .5 mol per liter dissolved phosphate, at least .3 mol per liter dissolved material from the group consisting of chromate and molybdate, and at least .2 mol per liter dissolved metal, and subsequently cold forming the coated billet to the desired predetermined shape.
2. The method as set forth in claim 1 wherein said solid particulate material consists at least in part of aluminum powder.
3. The method as set forth in claim 1 wherein said coating is heat cured at a temperature sufficient to cause

it to become water insoluble prior to said cold forming steps.

4. A method for forming a metal article of predetermined shape with a corrosion resistant coating thereon comprising the steps of coating a metal billet with a slurry of a solid particulate material in an aqueous solution, the solute of said aqueous solution consisting essentially of a combination of inorganic compounds selected from the group consisting of phosphoric acid, chromic acid, and the metal salts of said acids, the combination of compounds in said aqueous solution being such as will provide from about 1 to 4 mols per liter dissolved phosphate, from about .5 to 3 mols per liter dissolved chromate, and from about 1 to 4 mols per liter dissolved metal, heat curing said coating to cause it to become water insoluble and then cold forming the billet to the desired predetermined shape.

5. A method for forming a metal article of predetermined shape with a corrosion resistant coating thereon including the steps of cold forming to the desired predetermined shape, a metal billet coated with a dried and heat cured mixture of a solid particulate material and

an aqueous solution, the solute of said aqueous solution consisting essentially of a combination of inorganic compounds selected from the group consisting of phosphoric acid, chromic acid, molybdic acid, and the metal salts of said acids, the combination of compounds in said aqueous solution being such as will provide at least .5 mols per liter dissolved phosphate, at least .3 mols per liter dissolved material from the group consisting of chromate and molybdate, and at least .2 mols per liter dissolved metal.

References Cited by the Examiner

UNITED STATES PATENTS

|    |           |         |                 |       |          |
|----|-----------|---------|-----------------|-------|----------|
| 15 | 1,823,869 | 9/1931  | Baur            | ----- | 29—528   |
|    | 2,138,528 | 11/1938 | Phillipps       | ----- | 72—47    |
|    | 2,665,231 | 1/1954  | Amundsen et al. | ----- | 72—46    |
|    | 3,097,978 | 7/1963  | Newell et al.   | ----- | 148—6.16 |

20 CHARLES W. LANHAM, Primary Examiner.

L. A. LARSON, Assistant Examiner.